

## UNITED STATES PATENT OFFICE

1,926,614

## FIXATION OF DYES ON COLORED PAPER

Carl Z. Draves, Penns Grove, N. J., assignor to  
E. I. du Pont de Nemours & Company, Wil-  
mington, Del., a corporation of Delaware

No Drawing. Application July 24, 1931  
Serial No. 553,008

10 Claims. (Cl. 8—5)

This invention relates to a method for the fixation of the dyes on colored paper and more particularly to a method for rendering the dyes present on surface colored paper non-bleeding or relatively fast to the action of water and relates also to the resulting product.

In the art, it is often the practice to color paper after the sheet has been formed rather than by adding the dyestuff to the pulp when in the beater. This is accomplished either by dipping the sheet directly into a dye solution or by passing the sheet between rolls, one of which carries a film of dye solution to the surface of the paper. The dipping process is usually carried out in apparatus equipped with squeeze rolls for removing excess dye solution from the paper, although sometimes dipped sheets of paper are merely allowed to drain.

The method of coloring in which the dye solution is carried to the sheet upon the surface of a roll is often accomplished by placing dye boxes upon the calender stack in contact with the calender rolls. Coloring and calendering are thus accomplished in one operation and the process is known as calender dyeing.

Acid dyes are usually preferred for surface coloring because they possess great tintorial value and brightness of shade with satisfactory fastness to light. On the other hand, since the acid dyes have very little affinity for cellulose, they are held to the surface of the dry paper after it has been colored by any of the above processes merely by mechanical forces. Although direct dyes have much more real affinity for cellulose than acid dyes, paper which has been surface colored with direct dyes also bleeds much more than paper which has been dyed in the beater because much of the direct dye likewise is held to the surface merely by mechanical forces. When paper so colored comes into contact with water, a partial resolution of the dye occurs. This is objectional for two reasons: First, the appearance of the paper is harmed by the resulting spots and streaks; Second, any nearby object coming into contact with the paper in the presence of water is badly stained.

This invention has as an object the rendering of the dyestuff on surface colored paper relatively insoluble in water.

This object may be accomplished by the following invention. Paper, surface colored with acid or direct dyes either in the wet or dry state, is treated with diaryl guanidine in excess of the theoretical amount required to precipitate the dye. The complex formed by the diaryl guanidine

with the dye is relatively insoluble in water. However, the presence of excess diaryl guanidine causes more complete precipitation which results in less tendency for the dye to bleed.

My invention is generally applicable in connection with all dyes that are characterized by the presence of acid groups, such as, for example, the sulfonic acid or carboxyl groups, indeed to all dyes which give rise to colored anions when dissolved in aqueous solution. It is also in many cases of advantage to use a penetrating agent, such as, for example, methyl or ethyl alcohol or a higher alcohol.

The process may be applied to calender dyeing by placing a box upon the calender stack in such a position that the paper, after being coated with the dye solution contained in one box, is coated with diaryl guanidine solution contained in a second box. For example, the process may be satisfactorily applied in this manner to kraft lined container board. The dye solution containing 9 pounds 10 ounces of metanil yellow (C. I. No. 138) in 216 gallons of water is applied from the top box on the calender stack. An approximately 10% solution of diphenyl guanidine hydrochloride is prepared by pasting 6 pounds 10 ounces of diphenyl guanidine with 3 pounds 3 ounces of concentrated (38%) hydrochloric acid and diluting to eight gallons. This solution is applied continuously to the board from a lower box on the calender stack after the board has been colored from the box on an upper roll.

When surface dyed paper is dipped or calendered in a solution of diphenyl guanidine hydrochloride which contains enough free hydrochloric acid to be acid to Congo red, e. g. an excess of 4% over the amount necessary to form the hydrochloride, and is then heated in an oven at 100° C. for an hour, the tensile strength of the paper is decreased more than 25%. The tearing strength is probably decreased still more. It is therefore desirable to prepare the solution of the diaryl guanidine for after treatment in such a way that it does not contain an excess of strong acid.

Weak acids, such as acetic acid and hydrofluoric acid, possess the advantage for forming a soluble salt of the diaryl guanidine so that an excess of a weak acid exhibits less tendering action than a comparable excess of a strong, or highly ionized, acid. The character of the acid employed to dissolve the diaryl guanidine has nothing to do with the property of the diaryl guanidine in rendering the dye insoluble so long as the acid in question brings the free base into solution suf-

ficiently that it can react with the dye. Experiments show that dyed paper is not tendered because of after treatment with a salt of diaryl guanidine when the solution employed for after treatment is neutral in reaction, even when the salt is the hydrochloride.

It has been found that the hydrochloride of diphenyl guanidine can be conveniently prepared in the dry state by evaporation of the aqueous solution. The dry salt is not very hygroscopic and yet dissolves readily; it is convenient to handle and to ship and possesses the advantage of containing no excess acid even when the solution from which it is made by evaporation is slightly acid.

The dyestuff may be any acid or direct color or any combination of dyes from these two classes. Direct dyes form non-bleeding complexes upon treatment with solutions containing approximately one-eighth molecular weight of diaryl guanidine per liter of solution. Acid dyes require higher concentrations of the diaryl guanidine, varying from one-eighth molecular weight per liter to one molecular weight per liter. It will be understood that the amount of diaryl guanidine required to bring about a fairly complete precipitation of the dye, will vary with each individual case and is dependent upon the solubility of the complex formed, upon the number of acidic groups in the dye, upon the depth of shade of the dyeing, upon the absorbency of the paper, and upon the method by which the treatment is carried out. For these reasons the diaryl guanidine solution may vary in concentration from 0.5% for direct colors fixed by a dipping process to 25% for acid colors, the complex of which is relatively soluble, such as quinoline yellow Conc. (C. I. No. 801) and tartrazine O (C. I. No. 640) when fixed by the calendering process. A one-fourth molar solution of diaryl guanidine applied by the calendering method satisfactorily fixes any of the following direct dyes which have been applied to the surface of paper:

Du Pont brilliant paper yellow Conc. (C. I. No. 364), Du Pont stilbene yellow G Conc. (C. I. No. 622), pontamine fast scarlet 4BS (C. I. No. 326), pontamine fast red 8BL (C. I. No. 278), pontamine sky blue 6BX (C. I. No. 518), pontamine green GX (C. I. No. 594), pontamine black E (C. I. No. 581) et cetera.

Acid dyes such as pontacyl green NV Conc. (C. I. No. 735), pontacyl fast blue R (C. I. No. 208), pontacyl fast violet 10B (C. I. No. 696), Du Pont crocein scarlet N Extra (C. I. No. 252), and Du Pont metanil yellow Conc. (C. I. No. 138) may be satisfactorily rendered non-bleeding by coating sheets, surface colored with these dyes in moderately heavy shades, with a half molar solution of diaryl guanidine by the calendering process. Some acid dyes, such as pontacyl black SX (C. I. No. 246), Du Pont naphthol green B (C. I. No. 5), and pontacyl violet 4BL (C. I. No. 693), require a diaryl guanidine solution of lower concentration for fixation than the acid dyes mentioned above.

A greenish shade of grey paper, such as is used for wrapping papers, may be obtained by the use of a solution containing 1.33 oz. pontacyl blue black SX (C. I. No. 246), 0.37 ounces Du Pont metanil yellow Conc. (C. I. No. 138), and 0.46 ounces Du Pont crocein scarlet Conc. (C. I. No. 252), diluted to one gallon. Paper surface dyed with the above solution is rendered non-bleeding by passage between rolls one of which carries a

film of one-fourth molar diphenyl guanidine hydrochloride solution.

Any diaryl-guanidine may be employed as the fixing agent. Diphenyl, di-o-tolyl, di-o-anisyl, di-p-phenetyl, etc. may be utilized or triphenyl-guanidine may be employed. Further, any acid giving to the diaryl guanidine the required solubility in water may be used. Diphenyl guanidine hydrochloride is to be preferred on the basis of cost. Also, since the hydrochloride of diphenyl guanidine can be made into stock solutions containing as little as 10% water, it is more convenient to apply than the sulfate which has a much lower solubility in water. The acetate is very soluble in concentrated solutions, but hydrolyzes considerably upon being diluted to the proper concentrations for use in treating colored paper.

The above process may be modified by applying the fixing agent previous to the dye. Alcohol or other penetrating agents may be added to either dye or fixing solution. The free base of an aryl guanidine may be applied from an alcoholic solution if desired, although organic solutions possess the disadvantage of greater cost.

The paper may be given a double treatment of the fixing bath to secure less bleeding of the dyestuff. Any suitable method, such as dipping or a process analogous to calender dyeing may be used to apply the diaryl guanidine to the paper. The dyed paper may be either wet or dry when after-treated.

The invention may be used in fixing dyestuffs upon board, wrapping, tissue, crepe, absorbent, building, cardboard, cover, news, printing or writing papers. In general, the process is applicable to any surface dyed paper requiring water-fast colors.

The paper produced by the process here disclosed can be moistened with drops of water and the dye thereon will not spot or run from the paper as with surface dyed paper produced by the usual methods in which the water soluble dye is not rendered insoluble but is dried into the sheet and allowed to remain in its original form. The disadvantages of dyed paper from which the dye will bleed are that such paper when wet stains the hands or clothing or articles which may come in contact with it and that drops of water cause an unattractive spotting of the surface of the paper.

The aryl guanidines possess the great advantage over certain other organic bases, such as the naphthylamines, benzidine and 5-ethoxy-1-aminobenzothiazol which are also effective in preventing the bleeding of surface colored paper, that the aryl guanidines affect the fastness to light much less than other organic bases.

As many apparent and widely different embodiments of this invention may be made without departing from the spirit thereof, it is to be understood that I do not limit myself to the foregoing examples or descriptions except as indicated in the following claims.

I claim:

1. The method of coloring paper which comprises applying a dye containing an acid group thereto and fixing said dye by applying to the dyed paper a substance of the group consisting of di- and tri-aryl guanidines.

2. The method of coloring paper which comprises applying a dye containing an acid group thereto and fixing said dye by applying to the dyed paper a diaryl guanidine.

3. The method of coloring paper which comprises applying a dye containing an acid group

80

85

90

95

100

105

110

115

120

125

130

135

145

140

150

- thereto and fixing said dye by applying to the dyed paper diphenyl guanidine.
4. The method of coloring paper which comprises applying a dye containing an acid group thereto and fixing said dye by applying to the dyed paper diphenyl guanidine in concentration exceeding about one-eighth mol per liter.
5. The method of coloring paper which comprises applying a dye containing an acid group thereto and fixing said dye by applying to the dyed paper diphenyl guanidine in concentration from about 0.5 to 25 per cent.
6. The method of rendering dyed paper non-bleeding to water which comprises treating paper, dyed with a dye containing an acid group with a solution of a diaryl guanidine in excess of the theoretical amount necessary to precipitate the dye.
7. The method of preparing non-bleeding dyed paper which comprises treating paper with a penetrating agent, applying to said paper a diaryl guanidine in excess of the theoretical amount necessary to precipitate the dye and, in conjunction with the foregoing treatments, applying to said paper a dye containing an acid group.
8. Paper dyed with a dye containing an acid group of improved non-bleeding quality comprising a diaryl guanidine as a fixative.
9. Paper dyed with a dye containing an acid group of improved non-bleeding quality comprising diphenyl guanidine as a fixative.
10. Paper dyed with a dye containing an acid group of improved non-bleeding quality comprising diphenyl guanidine in excess of the theoretical amount necessary to precipitate the dye.

CARL Z. DRAVES.

Patent No. 1,926,614.

September 12, 1933.

CARL Z. DRAVES.

It is hereby certified that error appears in the printed specification of the above numbered patent requiring correction as follows: Page 3, lines 84, 87, and 90, claims 8, 9, and 10, respectively, after "group" insert the words and being; and that the said Letters Patent should be read with these corrections therein that the same may conform to the record of the case in the Patent Office.

Signed and sealed this 28th day of November, A. D. 1933.

F. M. Hopkins

(Seal)

Acting Commissioner of Patents.

- thereto and fixing said dye by applying to the dyed paper diphenyl guanidine.
4. The method of coloring paper which comprises applying a dye containing an acid group thereto and fixing said dye by applying to the dyed paper diphenyl guanidine in concentration exceeding about one-eighth mol per liter.
5. The method of coloring paper which comprises applying a dye containing an acid group thereto and fixing said dye by applying to the dyed paper diphenyl guanidine in concentration from about 0.5 to 25 per cent.
6. The method of rendering dyed paper non-bleeding to water which comprises treating paper, dyed with a dye containing an acid group with a solution of a diaryl guanidine in excess of the theoretical amount necessary to precipitate the dye.
7. The method of preparing non-bleeding dyed paper which comprises treating paper with a penetrating agent, applying to said paper a diaryl guanidine in excess of the theoretical amount necessary to precipitate the dye and, in conjunction with the foregoing treatments, applying to said paper a dye containing an acid group.
8. Paper dyed with a dye containing an acid group of improved non-bleeding quality comprising a diaryl guanidine as a fixative.
9. Paper dyed with a dye containing an acid group of improved non-bleeding quality comprising diphenyl guanidine as a fixative.
10. Paper dyed with a dye containing an acid group of improved non-bleeding quality comprising diphenyl guanidine in excess of the theoretical amount necessary to precipitate the dye.

CARL Z. DRAVES.

Patent No. 1,926,614.

September 12, 1933.

CARL Z. DRAVES.

It is hereby certified that error appears in the printed specification of the above numbered patent requiring correction as follows: Page 3, lines 84, 87, and 90, claims 8, 9, and 10, respectively, after "group" insert the words and being; and that the said Letters Patent should be read with these corrections therein that the same may conform to the record of the case in the Patent Office.

Signed and sealed this 28th day of November, A. D. 1933.

F. M. Hopkins

(Seal)

Acting Commissioner of Patents.

**CERTIFICATE OF CORRECTION.**

Patent No. 1,926,614.

September 12, 1933.

**CARL Z. DRAVES.**

It is hereby certified that error appears in the printed specification of the above numbered patent requiring correction as follows: Page 3, lines 84, 87, and 90, claims 8, 9, and 10, respectively, after "group" insert the words and being; and that the said Letters Patent should be read with these corrections therein that the same may conform to the record of the case in the Patent Office.

Signed and sealed this 28th day of November, A. D. 1933.

**F. M. Hopkins**

(Seal)

**Acting Commissioner of Patents.**